

Patented Dec. 8, 1953

2,662,024

*Leffman*

## UNITED STATES PATENT OFFICE

2,662,024

## CEMENTITIOUS COMPOSITIONS

Wallace C. Riddell, Berkeley, and George B. Kirk,  
Redwood City, Calif., assigners, by mesne assignments,  
to Kaiser Gypsum Company, Inc., a corporation of Washington

No Drawing. Application March 1, 1951,  
Serial No. 213,483

11 Claims. (CL 106—109)

1

This invention relates to cementitious compositions; and particularly to such compositions for use with gypsum wallboard, especially for filling the joints between panels and for smoothing the surfaces of the boards after installation.

In order to produce a monolithic effect in a construction using gypsum wallboard it is necessary to treat the joints between boards, nail heads and any other surface defects so that a smooth, uniform surface results. Cementitious or adhesive materials have been proposed for these purposes in the prior art, but have had some disadvantages. Many such compositions have had a protein base, for example, but this type of adhesive requires considerable waiting time, for instance, 20 to 30 minutes, after mixing the dry powder with water, to allow the protein to go into solution. In some commercial cements a marked change in consistency occurs during the waiting period so that it is necessary to readjust the consistency by mixing in more dry powder to obtain a workable paste. A strongly alkaline pH is also essential in employing such a material. This strongly alkaline condition is quite disadvantageous in application to wallboard because it is injurious to the paper covering of the board, resulting in weakening of the paper and marring its surface appearance. In other practices of the prior art, farinaceous substances have been employed in such compositions, but it has been necessary to use only small portions because of the increased tendency to cause cracks and checks in the surface, which remain even after the surface has been painted. The tendency to crack and check also occurs in the same manner with the protein-containing materials which also shrink appreciably in drying.

The above disadvantages are overcome by the cementitious composition of the present invention; and still further advantages are obtained. According to the present invention there is provided a cementitious composition, or a cement for forming joints between wallboards and for providing a smooth, uniform surface for wallboards, containing from 35% to 50% deadburned gypsum, from 15% to 20% of dextrin, from 5% to 10% of clay, from 10% to 20% of mica, from 10% to 20% of asbestos, and less than 1.0% of Portland cement. Preferably, the cementitious composition also contains from 0.5% to 2% of a dispersing agent, or from 0.2% to 1.0% of a wetting agent, or, advantageously, both of these ingredients. Alternatively, if desired, the wetting agent or the dispersing agent, or both, can be

2

added to the mixing water at the time and place of use of the composition.

The composition is employed as a finely divided powder, according to the usual good practice in this art. In use, it is mixed with water to a smooth paste and can be applied to the joint or surface immediately, e. g. in filling the joints between adjacent edges of wallboard or in covering nail heads or surface defects in the board. Any paste which remains unused at the end of a working day can be retempered, that is, mixed with water to the desired consistency, replacing water lost by evaporation, on the following day, and can be then employed in the same manner as freshly prepared paste. The cementitious paste is applied to the wallboard joint or surface and sets to a hard composition in a short time, for example in about 2 to 3 hours, depending on weather conditions, due in large part to setting of the dextrin component; upon further standing the deadburned gypsum or Keene's cement slowly sets also, forming a strong mass of interlaced gypsum crystals, providing still further increased strength, hardness, and water- and heat-resistance.

The deadburned gypsum employed is Keene's cement or other deadburned gypsum which sets very slowly and is not sensitive to atmospheric moisture. Keene's cement, for example, is well known to the art and comprises a gypsum calcined to a temperature of 1200° F. to 1600° F., which after calcining is ground to substantially pass a 100 mesh screen, and then usually a small amount of accelerator is added, for instance less than about 1% of aluminum sulfate or potassium sulfate, or of each when both are added. Such material, because it sets slowly in the cementitious composition, provides late and increased strength in finely divided form in order to provide a smooth surface when set. Suitably, this gypsum can be of a size to substantially entirely pass a 100 mesh screen. The dextrin component is, for example, a dextrinized starch or it can be a mixture of dextrin and a minor portion, up to about 15% of the weight of this component, of a partially dextrinized starch which, for example, can contain from 20% to 40% water-soluble constituents, or which contains from 15% to 25% water-soluble starch and dextrin calculated as starch. As an example of one partially dextrinized starch useful in this invention, such a material is employed which requires, per 100 grams thereof, 500 to 600 milliliters of water to form, upon mixing, a paste which will just pour. Mixtures of dextrin and such partially dextrin-

ized starch are particularly advantageous because they provide desired bulkiness. In a preferred embodiment, a dextrin component as described is employed which contains 17 parts by weight of dextrin and 3 parts by weight of partially dextrinized starch, or "modified corn flour" as it is sometimes known in the trade, these weights being based on the total weight of the joint cement mixture. The dextrin is a product made, for example, by treating corn starch with acid in a water medium, with heating, to convert to dextrin. After the conversion is finished, the fluid is neutralized, dried and ground. Starches other than corn starch can be employed in making the dextrinized or partially dextrinized product. The starchy component gives a much harder and stronger early set in the composition of this invention.

The clay employed is a plastic clay, preferably commercial fire clay, and is also used in finely divided form. It improves the workability of the paste so that it can be readily applied or "buttered onto" the surface to be treated.

Mica is also employed in finely divided form and it is of special advantage in a composition containing the hereinabove-defined amounts of dextrin component. The use of these high amounts of the dextrin component produces a strong and hard composition but, in the absence of the amount of mica defined, the dried cement exhibits shrinkage cracks or checking. It has been found that these cracks and checks are substantially entirely eliminated by the addition of the mica in the amounts shown, especially in cooperation with the amount of asbestos added. Furthermore, the adhesiveness of the composition is apparently improved by the mica addition. The asbestos fiber forms a fibrous mat in the composition which enables uniform drying of the composition with more uniform development of strength and desired surface characteristics, and aids in the prevention of cracking and checking upon drying.

A small amount of Portland cement, that is, less than 1.0%, and preferably from about 0.2% to about 0.3%, is included in the composition. This acts to maintain a slightly alkaline reaction, which is found to prevent rusting of nailheads in contact with the cement, but at the same time the alkalinity is maintained well below that which causes damage to paper, especially the paper liner or covering of gypsum wallboard. It is one theory of the operation of the Portland cement addition, but without intention of being limited by this theory, that this cement in the presence of water hydrolyzes slowly to form an amount of  $\text{Ca}(\text{OH})_2$  which maintains the desired alkalinity. At the same time Portland cement is stable when stored in air, whereas if an equivalent amount of calcium hydroxide were added in the mix, it would absorb carbon dioxide from the air to form the carbonate, reducing its effectiveness. The Portland cement in the composition of this invention is added in sufficient amount to maintain the alkalinity thereof at from more than pH 7.0 to less than pH 8.0, when in the presence of water.

Preferably a dispersing agent is also included with the cementitious composition of this invention. The dispersing agent can be included in the composition itself. Alternatively, excellent results can also be obtained by mixing the dispersing agent with the tempering water and then incorporating this into a paste with the composition as above described. The dispersing

agent is preferably waste sulfite liquor which can be employed as the liquor, or in the concentrated or the dried form or state. The waste sulfite liquor is obtained by digesting wood, to produce cellulose pulp, with calcium or magnesium bisulfite in the well known manner. Ammonia-base sulfite liquor is also useful in this invention. According to most authorities, the metal or other positive ion salt of the lignosulfonic acid is the effective constituent. In this specification and claims the agent will be termed "waste sulfite liquor." There can also be employed herein a purified lignin derivative of wood which has been digested with caustic soda or sodium sulfite, to produce cellulose pulp. This lignin derivative is preferably employed in the form of the water-soluble sodium salt. This lignin derivative and its sodium salt are described in a brochure entitled "Indulin: Lignin from Pine Wood," published by West Virginia Pulp & Paper Company. Alternatively, also, there can be employed in this invention a dispersing agent which is a water-soluble salt of a condensed aryl sulfonic acid, such as the sodium salt of condensed mononaphthalene sulfonic acid. The dispersing agent is preferably added in an amount of from about 0.5% to about 2.0% by weight, based on the total weight of the mix; and it can be added in the dry state, or an equivalent amount of liquid.

Preferably a wetting agent is also included with the above-described cementitious composition. The wetting agent can be included in the composition itself. Alternatively, the wetting agent can be incorporated in the tempering water, if desired, along with the dispersing agent described above, and this mixture can be added to the dry mixture of ingredients described above, to form the pasty mass for application to the wallboard joint or surface. The wetting agent is, for example, an alkyl aryl sulfonate, such as a sodium alkyl aryl sulfonate, an alkylated mono-sodium benzene sulfonate, or the like. Any other desired wetting agent can be employed. The wetting agent wets out the paper liner of the gypsum board, promoting bonding of the cement thereto. The wetting agent is preferably added in an amount of from about 0.2% to about 1.0% based on the total dry weight.

It is an advantage of the present invention that the composition sets fairly rapidly to give a hard cement with a high early strength; and another advantage is that the deadburned gypsum, or Keene's cement, sets more slowly providing continually increasing strength and a final very hard and strong product. It is believed that some of the Keene's cement combines with the sugars present in the dextrin or partially dextrinized starch to form insoluble calcium saccharate, which enhances the strength and hardness of the final product. It is a further and particular advantage of this composition that the incorporation of mica prevents cracking or checking so successfully that relatively large amounts of dextrin can be incorporated to give the enhanced early strength and hardness, and that the final surface is smooth and continuous, as desired. It is also an advantage that the material can be mixed with water and used immediately. Further advantages will be noted from the above description.

A specific example of a cementitious composition according to the present invention is as follows:

|                                                         |        |
|---------------------------------------------------------|--------|
| Keene's cement, substantially entirely passing 100 mesh | 47.00  |
| Dextrin                                                 | 17.00  |
| Partially dextrinized corn flour                        | 3.00   |
| Mica, powdered                                          | 15.00  |
| Asbestos fiber, finely ground                           | 10.00  |
| Fireclay, finely ground                                 | 7.00   |
| Portland cement                                         | 0.25   |
| Waste sulfite liquor (dry)                              | 0.50   |
| Wetting agent (alkyl aryl sulfonate)                    | 0.25   |
|                                                         | 100.00 |

10% to 20% of finely ground asbestos, a small amount of Portland cement and from 0.5% to 2% of a dispersing agent, said Portland cement being present in an amount of less than about 1%.

8. Cement for wallboard joints and surfaces containing from 35% to 50% finely divided dead-burned gypsum, from 15% to 20% of dextrin, from 5% to 10% of finely divided plastic clay, from 10% to 20% of finely divided mica, from 10% to 20% of finely ground asbestos, a small amount of Portland cement and from 0.2% to 1% of a wetting agent, said Portland cement being present in an amount of less than about 1%.

15 9. Cement for wallboard joints and surfaces containing from 35% to 50% finely divided dead-burned gypsum, from 15% to 20% of dextrin, from 5% to 10% of finely divided plastic clay, from 10% to 20% of finely divided mica, from 10% to 20% of finely ground asbestos, and a small amount of Portland cement, said Portland cement being present in an amount of less than about 1%, and having a pH of from more than 20 25 7.0 to less than 8.0 in the presence of water, said percentages being based on the total weight of the dry mixture.

20 10. Cement for wallboard joints and surfaces containing from 35% to 50% finely divided dead-burned gypsum, from 15% to 20% of dextrin, from 5% to 10% of finely divided plastic clay, from 10% to 20% of finely divided mica, from 10% to 20% of finely ground asbestos, a small amount of Portland cement, said Portland cement being present in an amount of less than about 1%, from 1% to 2% of a dispersing agent, and from 0.2% to 1% of a wetting agent, said percentages being based on the total weight of the mixture, said cement having a pH of from 25 30 35 40 45 50 more than 7.0 to less than 8.0 in the presence of water.

11. Cement for wallboard joints and surfaces containing 47% of Keene's cement substantially entirely passing 100 mesh, 15% finely divided mica, 10% finely ground asbestos fibers, 7% finely divided fire clay, 17% dextrin, 3% partially dextrinized corn starch, 0.5% dried waste sulfite liquor, 0.25% of a sodium salt of an alkyl aryl sulfonate and 0.25% of Portland cement, said percentages being based on the total weight of the mixture.

WALLACE C. RIDDELL.  
GEORGE B. KIRK.

55 References Cited in the file of this patent

UNITED STATES PATENTS

| Number    | Name      | Date          |
|-----------|-----------|---------------|
| 1,194,926 | Anderson  | Aug. 15, 1916 |
| 1,858,369 | Linzell   | May 17, 1932  |
| 1,863,990 | Nelson    | June 21, 1932 |
| 2,127,451 | Scripture | Aug. 16, 1938 |
| 2,318,540 | Talbert   | May 4, 1943   |
| 2,322,930 | Gardner   | June 29, 1943 |